

May 27, 1930.

H. C. RENTSCHLER ET AL

1,760,440

ELECTRON EMISSION MATERIAL

Original Filed June 25, 1921



INVENTORS

HARVEY C. RENTSCHLER  
JOHN W. MARDEN & CLAYTON T. ULRAY

BY

*J. J. Albert*  
ATTORNEY

## UNITED STATES PATENT OFFICE

HARVEY C. RENTSCHLER, JOHN W. MARDEN, AND CLAYTON T. ULREY, OF EAST ORANGE, NEW JERSEY, ASSIGNEES TO WESTINGHOUSE LAMP COMPANY, A CORPORATION OF PENNSYLVANIA

## ELECTRON-EMISSION MATERIAL

Original application filed June 25, 1921, Serial No. 480,301. Divided and this application filed December 23, 1922. Serial No. 608,784.

This application is a division of our application, Serial No. 480,301, filed June 25, 1921, for an improvement in Electron emission material, and assigned to the Westinghouse 5 Lamp Company.

This invention relates to electron-emission material and, more particularly, to refractory metals and alloys which have characteristics making them especially desirable for electron-emission.

Vacuum tubes for various purposes, such as for detectors and oscillators in wireless receiving and sending apparatus, are of considerable importance, and the material from 15 which the cathodes of such tubes are constructed generally determines the life and utility thereof. It is desirable that the cathode has a high electron emission, and it should be so designed as to be operated at as 20 low temperature as possible in order to avoid vaporization of the material thereof, since such vaporization causes rapid deterioration of the cathode and decreases the life of the tube. The use of lower temperatures also results in a higher electrical efficiency of the 25 tube.

Various types of cathodes and various kinds of materials therefore have been proposed and, although they are fairly successful, the efficiency and operating characteristics thereof are not entirely satisfactory because of the high operating temperatures. It has been proposed to utilize tungsten filaments, or metal coated with various oxides, 30 such as oxides of calcium, strontium, barium or the like. In order to obtain a suitable electron emission from tungsten filaments, it is necessary to operate the cathode at such high temperature that the life of the bulb is relatively short and the bulb becomes blackened 40 very rapidly. The oxide coated filaments disintegrate and develop hot spots, causing the burning out of the cathode at such spots.

Our invention contemplates the production 45 of an electron-emission material which is far superior to any proposed heretofore, which may be operated at much lower temperatures, giving a greater electron emission and having a higher efficiency.

50 In practicing our invention, we utilize rare

metals. We have found that uranium has an electron emission at comparatively low temperatures which is equal to the electron emission of tungsten at temperatures of about 325° C. higher.

Our material consists essentially of the refractory metal uranium, which has a high electron-emissive power and, in order to modify its properties to make it more suitable for filaments, we may alloy it with another 60 metal, for instance, tungsten, to improve its working properties.

The accompanying drawing illustrates curves obtained by plotting the milliamperes of current produced by one square centimeter of electron-emission material as ordinates, against temperatures as abscissæ.

It will be seen that the curve for uranium is of approximately the same type as that for tungsten with the exception that it is placed at 70 a point at about 325° C. lower than the tungsten curve. The uranium materials give electron emissions at about 1700° C. of the same order as tungsten at about 2025° C.

Alloys of various refractory rare metals 75 also show high electron emission, particularly the uranium alloys. For instance, a uranium alloy of a composition containing 7% uranium and 93% tungsten shows an electron emission equal to that of a filament of pure uranium. 80 An alloy of 25% uranium and 75% tungsten also shows an electron emission substantially that of uranium. Alloys of uranium with metals, such as tungsten, molybdenum or tantalum, all show electron emissions superior to 85 that of the alloying metal, usually in the neighborhood of the electron emission of uranium.

We conclude, from these phenomena, that the electron-emitting power of a substance containing two or more elements is primarily a property of the electron emission of the element which is active at the lower temperatures, although this property may be modified to some extent by the molecular or physical structure of the material.

We claim as our invention:

1. Material suitable for use as an electron emitter in electron discharge devices comprised of a refractory metal body containing 100

approximately 93 per cent tungsten and approximately 7 per cent uranium.

2. In an electron discharge device employing a thermionic cathode and at least one co-  
5 operating electrode, a refractory hot cathode comprised of tungsten containing approxi-  
mately 7 per cent uranium alloyed there-  
with.

In testimony whereof, we have hereunto  
10 subscribed our names this 22nd day of  
December, 1922.

HARVEY C. RENTSCHLER.

JOHN W. MARDEN.

CLAYTON T. ULREY.

15

20

25

30

35

40

45

50